



US005948608A

# United States Patent [19]

Inagaki et al.

[11] Patent Number: **5,948,608**[45] Date of Patent: **Sep. 7, 1999**

## [54] PHOTOTHERMOGRAPHIC MATERIAL

[75] Inventors: **Yoshio Inagaki; Toyohisa Oya; Katsumi Kobayashi; Hirohiko Tsuzuki**, all of Ashigara, Japan

[73] Assignee: **Fuji Photo Film Co., Ltd.**, Kanagawa, Japan

[21] Appl. No.: **08/840,715**

[22] Filed: **Apr. 25, 1997**

## [30] Foreign Application Priority Data

Apr. 25, 1996 [JP] Japan ..... 8-105788

[51] Int. Cl.<sup>6</sup> ..... **G03C 1/498**

[52] U.S. Cl. ..... **430/619**; 430/584

[58] Field of Search ..... 430/584, 619

[56]

## References Cited

## U.S. PATENT DOCUMENTS

593,654 2/1897 Burrows et al. ..... 430/584  
5,597,279 1/1997 Mifune et al. ..... 430/567  
5,677,121 10/1997 Tsuzuki .

Primary Examiner—Thorl Chea  
Attorney, Agent, or Firm—Birch, Stewart, Kolasch & Birch,  
LLP

[57]

## ABSTRACT

A photothermographic material comprising light-sensitive silver halide grains, with the photosensitive material further comprising a heptamethine cyanine dye containing at least one arylthio or thienyl group as substituent.

**14 Claims, No Drawings**

## PHOTOTHERMOGRAPHIC MATERIAL

## FIELD OF THE INVENTION

The present invention relates to a photothermographic material.

## BACKGROUND OF THE INVENTION

In the field of clinical photography, a reduction in the quantity of processing waste has recently been desired from the viewpoint of environmental preservation and space saving. Thus, it has been required to develop the technology concerning photosensitive photothermographic materials which can achieve great effects in the exposure with a laser imagesetter or laser imager and produce clear black images having high resolution to enable use as clinical photographs for assisting diagnosis and medical treatment. With such photosensitive photothermographic materials, the use of processing chemicals of solution type can be made needless and a simpler heat-development processing system causing no damage to the environment can be afforded to customers.

On the other hand, the semiconductor laser technology which has made expeditious progress in recent years enables the miniaturization of a medical image-output unit. As a matter of course, there have been developed the arts of producing infrared-sensitive (light- and heat-sensitive) silver halide photographic materials which make it possible to use a semiconductor laser as light source. More specifically, the spectral sensitization arts applied to such photographic materials are disclosed in JP-B-03-10391 (The term "JP-B" as used herein means an "examined Japanese patent publication"), JP-B-06-52387, JP-A-05-341432 (The term "JP-A" as used herein means an "unexamined published Japanese patent application"), JP-A-06-194781 and JP-A-06-301141, and the anti-halation arts applied thereto are disclosed in JP-A-07-13295 and U.S. Pat. No. 5,380,635. In the photosensitive materials produced with a view to exposure to infrared rays, the absorption of visible rays by sensitizing dyes and anti-halation dyes can be reduced to a great extent, so that it is easy to render such photosensitive materials colorless in a substantial sense.

However, dyes capable of producing a spectral sensitization effect by the absorption of infrared rays generally have strong reducing power because of their high "HOMO", so that they are liable to worsen the photographic fog by reducing the silver ions in a photosensitive material. In particular, such dyes have a problem of causing a marked change in photographic properties upon storage under a high temperature-high humidity condition or upon long-term storage. Conversely, the dyes of low "HOMO" employed for preventing the deterioration in keeping properties are inferior in spectral sensitizing efficiency because they are comparatively low in "LUMO", so that the photosensitive materials containing those dyes are low in sensitivity. Not only the photographic materials of wet process type encounter the problems concerning the sensitivity and the keeping properties as mentioned above, but also those problems become more serious in photothermographic materials relating to the present invention.

In addition, it is natural that the reducing power produced by a dye has a tendency to be enhanced with an increase in the dye content. However, a decrease in the dye content causes a shortage of the sensitivity because the photosensitive material having a low dye content cannot sufficiently absorb the light incident thereon. In particular, photosensitive photothermographic materials using highly lipophilic binders are deficient in sensitivity unless dyes are added

thereto in sufficient amounts, because the adsorption of dyes to silver halide as a photosensitive element is weak therein.

## SUMMARY OF THE INVENTION

Therefore, an object of the present invention is to provide an infrared-sensitive photothermographic material having satisfactory keeping properties, low fog and high sensitivity.

The above object of the present invention is attained with the means described below:

(1) A photothermographic material containing light-sensitive silver halide grains on at least one side of a support, with the photothermographic material comprising a cyanine dye represented by the following formula (I):



wherein  $Z_1$  and  $Z_2$  each represents an atomic group for completing a benzene or naphthalene ring;  $Y_1$  and  $Y_2$  each represents O, S, Se or NR, wherein R is an alkyl group;  $R_1$  and  $R_2$  each represents an alkyl group;  $R_3$ ,  $R_4$ ,  $R_5$ ,  $R_6$ ,  $R_7$ ,  $R_8$  and  $R_9$  each represents a hydrogen atom or a substituent group, at least one pair of  $R_4$  and  $R_6$ ,  $R_5$  and  $R_7$ , and  $R_6$  and  $R_8$  may be combined with each other to complete a 5- or 6-membered ring, and  $R_4$ ,  $R_6$  and  $R_8$  may be combined with each other to form a condensed ring in which two 6-membered rings are fused; X represents a counter ion for adjusting the charge balance; i represents 0 or 1; provided that  $R_1$ ,  $R_2$ ,  $R_3$ ,  $R_4$ ,  $R_5$ ,  $R_6$ ,  $R_7$ ,  $R_8$ ,  $R_9$ ,  $R$ ,  $Z_1$  or  $Z_2$  contains as a substituent at least one thienyl or arylthio group.

(2) A photothermographic material having on at least one side of a support a binder, an organic silver salt, a reducing agent for silver ions and light-sensitive silver halide grains, with the photothermographic material comprising a cyanine dye of formula (I) illustrated above.

(3) A photothermographic material as described (1) or (2), with the light-sensitive silver halide grains being spectrally sensitized in the wavelength region of 750 to 1,400 nm.

## DETAILED DESCRIPTION OF THE INVENTION

In the compound represented by the present formula (I), it is desirable that the substitution position of a thienyl or arylthio group be  $Z_1$  or  $Z_2$ , or any of the substituents  $R_1$  to  $R_9$ , especially  $Z_1$  or  $Z_2$ .

The alkyl group represented by R,  $R_1$  and  $R_2$  each is preferably a straight-chain, branched or cyclic alkyl group containing 1 to 22 carbon atoms, which may further have a substituent. As examples of such a substituent, mention may be made of not only a thienyl group and an arylthio group but also a halogen atom (F, Cl, Br, I), a hydroxyl group, a carboxyl group, a  $C_2$ - $C_{20}$  alkoxy carbonyl group, a  $C_2$ - $C_{20}$  acyl group, a  $C_2$ - $C_{20}$  acyloxy group, a  $C_1$ - $C_{20}$  carbonamido group, a  $C_1$ - $C_{20}$  carbamoyl group, a  $C_1$ - $C_{20}$  alkoxy group, a  $C_6$ - $C_{10}$  substituted phenyl group, an unsubstituted phenyl group and a  $C_1$ - $C_{20}$  alkylthio group. As for the groups preferred as R,  $R_1$  and  $R_2$ , unsubstituted straight-chain alkyl groups containing 1 to 8 carbon atoms, carboxyalkyl groups containing 2 to 8 carbon atoms, alkylthioalkyl groups containing 2 to 8 carbon atoms, thienylalkyl groups containing

5 to 10 carbon atoms and arylthioalkyl groups containing 7 to 10 carbon atoms are examples thereof.

The thiienyl group contained as a substituent is a 2-thienyl group or a 3-thienyl group, which may further have a substituent. Suitable examples of such a substituent include an alkyl group containing 1 to 6 carbon atoms, a substituted phenyl group containing 6 to 10 carbon atoms (the substituent of which is preferably a halogen atom, an alkoxy group, an alkyl group, an alkylthio group, a carboxyalkyl group or a carboxy group), an unsubstituted phenyl group, an alkoxy group containing 1 to 6 carbon atoms, an alkylthio group containing 1 to 6 carbon atoms and a halogen atom (F, Cl, Br, I).

The arylthio group contained as a substituent is preferably a substituted phenylthio group containing 6 to 10 carbon atoms (the substituent of which is preferably a halogen atom, an alkoxy group, an alkyl group, an alkylthio group, a carboxyalkyl group or a carboxy group) or an unsubstituted phenylthio group. Such a thiaryl or arylthio group is preferably present as a substituent of the group represented by  $Z_1$ ,  $Z_2$ ,  $R_1$  or  $R_2$ .

The benzene or naphthalene ring completed by  $Z_1$  and  $Z_2$  each may further have a substituent. Suitable examples of such a substituent include not only the foregoing thiaryl and arylthio groups but also an alkyl group containing 1 to 6 carbon atoms, a substituted phenyl group containing 6 to 10 carbon atoms (the substituent of which is preferably a halogen atom, an alkoxy group, an alkyl group, an alkylthio group, a carboxyalkyl group or a carboxy group), an unsubstituted phenyl group, an alkoxy group containing 1 to 6 carbon atoms, an alkylthio group containing 1 to 6 carbon atoms and a halogen atom (F, Cl, Br, I). The fused position in the naphthalene ring completed by  $Z_1$  and  $Z_2$  each may be any of [1,2-d], [2,3-d] and [3,4-d].

Suitable examples of a substituent group represented by  $R_3$ ,  $R_4$ ,  $R_5$ ,  $R_6$ ,  $R_7$ ,  $R_8$  and  $R_9$  each include an alkyl group containing 1 to 8 carbon atoms, an alkoxy group containing 1 to 8 carbon atoms, an unsubstituted phenyl group, a substituted phenyl group containing 6 to 10 carbon atoms (the substituent of which is preferably a halogen atom, an alkoxy group, an alkyl group, an alkylthio group, a carboxy-alkyl group or a carboxy group), an unsubstituted phenoxy group, a substituted phenoxy group containing 6 to 10 carbon atoms, an aralkyl group containing 7 to 11 carbon atoms, an unsubstituted amino group, a substituted amino

group (e.g., dimethylamino, diphenylamino, morpholino, 4-acetyl piperazinyl) and a nitrogen-containing aromatic heterocyclic group (e.g., 1-pyrazolyl, 1-imidazolyl). As for  $R_3$  and  $R_6$ , they each prefer a hydrogen atom in particular.

The 5- or 6-membered ring completed by combining  $R_4$  with  $R_6$ , or  $R_5$  with  $R_7$ , or  $R_6$  with  $R_8$  is a carbon ring or a heterocyclic ring containing an oxygen, sulfur or nitrogen atom as a hetero atom, and may further have a substituent. Suitable examples of such a substituent include an alkyl group containing 1 to 4 carbon atoms, an alkoxy group containing 1 to 4 carbon atoms, an unsubstituted phenyl group, a substituted phenyl group containing 6 to 10 carbon atoms (the substituent of which is preferably a halogen atom, an alkoxy group, an alkyl group, an alkylthio group, a carboxyalkyl group or a carboxy group), an unsubstituted amino group, a substituted amino group (e.g., dimethylamino, diphenylamino, morpholino, 4-acetylpirazinyl) and a nitrogen-containing aromatic heterocyclic group (e.g., 1-pyrazolyl, 1-imidazolyl).

The counter ion represented by X is a cation or anion chosen so as to adjust the total charge of the compound of formula (I) to zero, and it may be present as a substituent on  $Z_1$ ,  $Z_2$ , R,  $R_1$ ,  $R_2$  or the like.

As for the cation suitable for X,  $\text{Na}^+$ ,  $\text{K}^+$ ,  $\text{NH}_4^+$ ,  $(n\text{-C}_4\text{H}_9)_4\text{N}^+$  and N-ethylpyridinium ion are examples thereof. As examples of an anion suitable for X, mention may be made of acid anions, such as chloride, bromide, iodide, tetrafluoroborate, hexafluorophosphate, methylsulfate, ethylsulfate, 4-methylbenzenesulfonate, 4-chlorobenzenesulfonate, benzenesulfonate, methanesulfonate and trifluoromethanesulfonate.

As for a desirable combination of structural sections in the compound of formula (I), there can be instanced the combination in which  $Z_1$  and  $Z_2$  each are atoms completing a benzene ring having a thiaryl or arylthio group, at least either  $Y_1$  or  $Y_2$  is S and the remainder is O or S, preferably both of them are S,  $R_1$  and  $R_2$  each are an unsubstituted alkyl group containing 2 to 6 carbon atoms or a carboxyalkyl group, and at least either the combination of  $R_4$  with  $R_6$  or the combination of  $R_6$  with  $R_8$  completes a 5- or 6-membered ring by coupling with each other.

Specific examples of a cyanine dye represented by formula (I) used in the present invention are illustrated below, but these examples should not be construed as limiting the scope of the invention in any way.

1



-continued

2.



3.



4.



5.



6.



-continued

7.



8.



9.



10.



11.



12.



5,948,608

**9****10**

-continued

13.



14.

I<sup>-</sup>

15.



16.



17.

I<sup>-</sup>

-continued

18.



19.



20.



21.



22.



23.



-continued

24.



25.



26.



27.



28.



29.



-continued

30.



31.



32.



33.



34.



35.



The present compounds represented by formula (I) or (II) can be synthesized according to the methods described in the following books or the references cited therein. Those books are, e.g., F. M. Hamer, *The Cyanine Dyes and Related Compounds*, from page 55 on, Interscience Publishers, New York (1964); Nikolai Tyutyulkov, Jurgen Fabian, Achim Ulehlhorn, Flitz Dietz & Alia Tadjer, *Polymethine Dyes*, pages 23–38, St. Kliment Ohridski University Press, Sophia; D. M. Sturmer, *Heterocyclic Compounds—Special Topics in Heterocyclic Chemistry*, Chapter 18, Section 14, pages 482–515, John Wiley & Sons Co., New York, London (1977); and Rodd's *Chemistry of Carbon Compounds*, 2nd Ed. Vol. IV, Part B, Chapter 15, pages 269–422 (1977), and 2nd Ed. Vol. IV, Part B, Chapter 15, pages 267–296 (1985), Elsvier Science Public Company Inc., New York.

Methods of synthesizing the present compounds represented by formula (I) are illustrated below by taking actual synthesis examples.

50

## Synthesis Example 1: Synthesis of Compound 12

A mixture of 3 g of 5-phenylthiobenzothiazole with 3.5 g of ethyl p-toluenesulfonate was heated at 150° C. for 5 hours, and then cooled to room temperature. Thereto, 150 ml of ethyl acetate was added with stirring. A 1.1 g portion of the thus deposited viscous matter was admixed with 1.05 g of glutaconic aldehyde dianil hydrochloride, and heated to 50° C. in ethanol with stirring. Thereto, 0.74 ml of triethylamine was added, and the stirring was continued for 1 hour. After cooling to room temperature, the reaction mixture was admixed with a solution containing 0.36 g of sodium iodide in methanol. The crystals thus formed were filtered off, and recrystallized from methanol to yield 130 mg of Compound 12.

$\lambda_{MAX}=774.3$  nm ( $\epsilon_{MAX} 2.54 \times 10^5$ ).

## Synthesis Example 2: Synthesis of Compound 1

To 40 ml of ethanol, 3 g of 3-ethyl-2-methyl-5-thienylbenzothiazolium p-toluenesulfonate and 2 g of N-[5-

(phenylamino)-2,4-pentadienylene]aniline hydrochloride were added, and heated to 50° C. to make a suspension. This suspension was admixed with 1 g of triethylamine, and stirred for 45 minutes at 50° C. to deposit crystals. These crystals were filtered off, and washed with ethanol. Thus, 2 g of crude crystals were obtained. These crude crystals were added to 500 ml of ethanol, and dissolved therein by heating. Thereto, a solution containing 1.5 g of sodium iodide in 50 ml of methanol was added to precipitate crystals having metallic luster. These crystals were filtered off, and washed with hot methanol to yield 1.6 g of Compound 1.

$$\lambda_{MAX}(\text{methanol})=777 \text{ nm } (\epsilon=2.7 \times 10^5).$$

It is desirable that the present cyanine dyes represented by formula (I) be used in an amount of from  $10^{-6}$  to 1 mole, preferably from  $10^{-5}$  to  $10^{-2}$  mole, per mole of silver halide.

The present cyanine dyes may be added to a light-sensitive silver halide emulsion at any stage in its preparation from the silver halide formation to just before the coating of the emulsion. Preferably, they are added just before the coating of the emulsion.

Also, the present cyanine dyes can be used as a mixture of two or more thereof to provide a desired spectral sensitization spectrum.

The present light-sensitive silver halide emulsion for heat development is applied to a support in the form of single or multiple layer. At least one constituent layer of the emulsion layer must comprise silver halide, and it is desirable for the constituent layer to further comprise the ingredients requested, such as an organic silver salt, a developer, a binder and auxiliary agents including a toning agent and a coating aid. When the emulsion layer has a double-layer structure, an organic silver salt and silver halide are contained in the first emulsion layer (which is generally adjacent to a support), while other ingredients besides those silver salts are contained in the second layer or in both the first and second layers. Further, the double-layer structure may be made up of a single emulsion layer containing all the ingredients and a protective top coat. With respect to the structure of a multicolor light-sensitive photothermographic material, either combination of two layers as mentioned above may be employed for each color, or a single layer may contain all the ingredients as described in U.S. Pat. No. 4,708,928. In a many dyes-added multicolor light-sensitive photothermographic material, as described in U.S. Pat. No. 4,460,681, each emulsion layer is generally held distinguishably from any other emulsion layer by providing a functional or non-functional barrier layer between every adjacent light-sensitive layers.

In order to achieve the desired spectral sensitization spectrum, the sensitizing dyes according to the present invention can also be used as the mixture of two or more thereof.

Besides the present sensitizing dyes having the structural formulae (I), other sensitizing dyes may be used together. Of the dyes usable together with the present sensitizing dyes, those which can confer spectral sensitivities upon silver halide grains at some wavelengths in the range of 750 nm to 1,400 nm by the adsorption to the silver halide grains are preferable. Specifically, various known dyes, including cyanine dyes, merocyanine dyes, styryl dyes, hemicyanine dyes, oxonol dyes, hemioxonol dyes and xanthene dyes, can be used to advantage in spectrally sensitizing light-sensitive

silver halide. As for the cyanine dyes, those having basic nuclei, such as thiazoline, oxazoline, pyrrolidine, pyridine, oxazole, thiazole, selenazole and imidazole nuclei, are useful. As for the useful merocyanine dyes, acidic nuclei such as thiohydantoin, rhodanine, oxazolidinedione, thiazolinedione, barbituric acid, thiazolinone, malononitrile and pyrazolone nuclei are contained therein in addition to the basic nuclei as recited above. Of the foregoing cyanine and merocyanine dyes, those containing imino or carboxyl groups are especially effective. More specifically, the dyes used together with the present sensitizing dyes may be properly selected from the known dyes as described in U.S. Pat. Nos. 3,761,279, 3,719,495 and 3,877,943, British Patents 1,466,201, 1,469,117 and 1,422,057, JP-B-03-10391, JP-B-06-52387, JP-A-05-341432, JP-A-06-194781 and JP-A-06-301141. In general, such dyes can be used in an amount of from about 10  $\mu\text{mole}$  to about 1 mole per mole of silver halide. Additionally, those dyes also can be used as a mixture of two or more thereof for the achievement of the desired spectral sensitization.

It is desirable for the present photothermographic material to be a photosensitive material which has on one side thereof at least one light-sensitive layer comprising a silver halide emulsion and on the other side a backing layer, namely the so-called single-sided photosensitive material.

In forming the light-sensitive silver halide contained in the present photothermographic material, methods well known in the art, e.g., the methods described in *Research Disclosure*, No. 17029 (June, 1978) and U.S. Pat. No. 3,700,458, can be adopted. More specifically, the present invention can employ the method of adding a halogen-containing compound to the prepared organic silver salt to convert a part of the silver of the organic silver salt into the light-sensitive silver halide, or the method of preparing light-sensitive silver halide grains by the addition of a silver-supplying compound and a halogen-supplying compound to a solution of gelatin or another polymer and then mixing the prepared grains with an organic silver salt. In particular, the latter method is preferred in the present invention. As for the light-sensitive silver halide, smaller grains are desirable from the viewpoint of preventing the photosensitive material from becoming clouded after the image formation. Specifically, it is desirable for the grain size to be not greater than 0.20  $\mu\text{m}$ , preferably from 0.01 to 0.15  $\mu\text{m}$ , particularly preferably from 0.02 to 0.12  $\mu\text{m}$ . The term "grain size" used herein signifies "edge length" when the grains have a regular crystal form such as a cubic or octahedral form. In the case of tabular silver halide grains, the term "grain size" refers to the diameter of the circle having the same area as the projected area of the main face of each tabular grain. In cases where the silver halide grains have irregular crystal forms, such as spherical and rod-like forms, the term "grain size" means the diameter of the sphere having the same volume as each grain.

With respect to the form of silver halide grains, a cubic form, an octahedral form, a tabular form, a spherical form, a rod-like form and a potato-like form are examples thereof. In particular, cubic grains and tabular grains are preferred over the others in the present invention. When tabular silver halide grains are employed, it is desirable for the average aspect ratio thereof to be from 100 to 2, preferably from 50

to 3. Also, silver halide grains having round corners are preferably used in the present invention. The light-sensitive silver halide grains used in the present invention has no particular restriction as to the Miller indices of their outer surfaces. However, it is desirable that [100] plane be present in a high proportion, because a spectral sensitizing dye adsorbed to that plane has high spectral sensitizing efficiency. The appropriate proportion of [100] plane is not lower than 50%, preferably at least 65%, particularly preferably at least 80%. The proportion of [100] plane can be determined using the method described in T. Tani, *J. Imaging Sci.*, 29, 165 (1985), wherein the difference between [111] plane and [100] plane in the adsorption of a sensitizing dye thereto is utilized. The light-sensitive silver halide used in the present invention has no particular restriction on halide composition, so that it may be any of silver chloride, silver chlorobromide, silver bromide, silver iodobromide, silver iodochlorobromide and silver iodide. However, silver bromide or silver iodobromide can be advantageously used in the present invention, wherein the suitable iodide content is from 0.1 to 40 mole %, preferably from 0.1 to 20 mole %. The halide composition may have a uniform distribution inside the grains, or it may change stepwise or continuously inside the grains. For instance, it is favorable to use silver iodobromide grains having a higher iodide content in the inner part thereof or silver halide grains having a core/shell structure. As for the grains having a core/shell structure, the core/shell grains having a double to quintuple structure, preferably a double to quadruple structure, can be used to advantage.

Further, it is desirable for the light-sensitive silver halide grains used in the present invention to contain at least one metal complex selected from the group consisting of rhodium complexes, rhenium complexes, ruthenium complexes, osmium complexes, iridium complexes, cobalt complexes and iron complexes. These metal complexes may be used alone or as a mixture of two or more of different complexes whose metal components may be the same or different. The suitable content of such metal complexes is from 1 nmole to 10 mmole, preferably from 10 nmole to 100  $\mu$ mole, per mole of silver. With the respect to specific structures of such metal complexes, the metal complexes having the structures described in JP-A-07-225449 can be used to advantage. Of the cobalt complexes and iron complexes, hexacyanocobaltates and hexacyanoferrates are preferred over others. More specifically, ferricyanate ion, ferrocyanate ion and hexacyanocobaltate ions are used to advantage, but the metal complexes usable in the present invention should not be construed as being limited to those ions. The metal complexes as mentioned above may be incorporated uniformly in each silver halide grain or in a higher concentration in the core part than the shell part of each silver halide grain. There is no particular restriction on the way of incorporating those metal complex, though.

The light-sensitive silver halide grains can be desalts by the washing treatment according to a method well known in the art, such as a noodle method or a flocculation method. However, such a desalting process may be omitted in the present invention.

Furthermore, it is desirable that the light-sensitive silver halide grains used in the present invention be chemically

sensitized. For the chemical sensitization, as well known in the art, a sulfur sensitization method, a selenium sensitization method and a tellurium sensitization method can be employed. Also, a precious metal sensitization method using a gold, platinum, palladium or iridium compound and a reduction sensitization method can be adopted. Although the compounds known to be suitable for sulfur, selenium and tellurium sensitization methods can be used in the present invention also, the compounds described in JP-A-07-128768 can be used to greater advantage. As for the tellurium sensitizer, diacytellurides, bis(oxycarbonyl)tellurides, bis(carbamoyl)tellurides, bis(oxycarbonyl)ditelluride, bis(carbamoyl)ditellurides, the compounds having P=Te bonding, tellurocarboxylates, Te-organyl tellurocarboxylic acid esters, di(poly)tellurides, tellurides, tellurols, telluroacetals, tellurosulfonates, the compound having P-Te bonding, tellurium-containing heterocyclic rings, tellurocarboxylic compounds, inorganic tellurium compounds and colloidal tellurium are specific examples thereof. As for the compounds suitably used for a precious metal sensitization method, chloroauric acid, potassium chloroaurate, potassium aurithiocyanate, gold sulfide, gold selenide and the compounds described in U.S. Pat. No. 2,448,060 and British Patent 618,061 are specific examples thereof. As specific examples of a compound suitable for reduction sensitization, mention may be made of ascorbic acid, thiourea dioxide, stannous chloride, aminoiminomethanesulfonic acid, hydrazine derivatives, borane compounds, silane compounds and polyamine compounds. In addition, the reduction sensitization can be effected by ripening emulsions under the pH of above 7 or the pAg of below 8.3. Also, the reduction sensitization can be attained by introducing the stage of single addition of silver ion in the course of the grain formation.

The amount of light-sensitive silver halide used in the present invention is preferably from 0.01 to 0.5 mole, more preferably from 0.02 to 0.3 mole, particularly preferably from 0.03 to 0.25 mole, per mole of organic silver salt. With respect to the way of and the condition for mixing the light-sensitive silver halide with an organic silver salt, the silver halide grains and the organic silver salt prepared independently may be mixed by means of a high-speed stirrer, a ball mill, a sand mill, a colloidal mill, a vibration mill, a homogenizer or the like, or the silver halide grains prepared separately may be added at due time during the preparation of an organic silver salt to prepare a mixture of the silver halide with the organic silver salt. However, the present invention has no particular restriction as to the mixing method and condition so far as the effects intended by the invention can be fully achieved.

The organic silver salts usable in the present invention are silver salts which, although they are relatively stable to light, can provide silver images when they are heated to 80° C. or higher in the presence of an exposed photocatalyst (e.g., a latent image formed from light-sensitive silver halide) and a reducing agent. And the organic silver salts may be any of organic substances containing roots capable of reducing silver ion. Of such silver salts, the silver salts of organic acids, especially the silver salts of long-chain aliphatic carboxylic acids (containing 10 to 30, preferably 15 to 28, carbon atoms), are used to advantage. In addition, the

complexes of organic or inorganic silver salts whose ligands have complexation stability constants ranging from 4.0 to 10.0 are also favorable. The silver providing substances can preferably constitute about 5 to 30 weight % of the image-forming layer. The desirable organic silver salts include the silver salts of organic compounds containing carboxyl groups, wherein the silver salts of aliphatic carboxylic acids and those of aromatic carboxylic acids are included. However, the organic silver salts usable in the invention should not be construed as being limited to those salts. Suitable examples of a silver salt of aliphatic carboxylic acid include silver behenate, silver stearate, silver oleate, silver laurate, silver caproate, silver myristate, silver palmitate, silver maleate, silver fumarate, silver tartarate, silver linolate, silver butyrate, silver camphorate and a mixture of two or more thereof.

Also, the silver salts of mercapto or thione group-containing compounds and derivatives thereof can be used. Suitable examples thereof include the silver salt of 3-mercaptopro-4-phenyl-1,2,4-triazole, the silver salt of 2-mercaptopbenzimidazole, the silver salt of 2-mercaptop-5-aminothiadiazole, the silver salt of 2-(ethylglycolamido)benzothiazole, the silver salts of thioglycolic acids, such as a silver S-alkylthioglycolate (the alkyl moiety of which contains 12 to 22 carbon atoms), the silver salts of dithiocarboxylic acids, such as silver dithioacetate, the silver salts of thioamides, the silver salt of 5-carboxy-1-methyl-2-phenyl-4-thiopyridine, the silver salt of mercaptotriazine, the silver salt of 2-mercaptopbenzoxazole, the silver salts described in U.S. Pat. No. 4,123,274 including the silver salts of 1,2,4-mercaptopthiazole derivatives, such as the silver salt of 3-amino-5-benzylthio-1,2,4-thiazole, and the silver salts described in U.S. Pat. No. 3,301,678 including the silver salts of thione compounds, such as the silver salt of 3-(3-carboxyethyl)-4-methyl-4-thiazoline-2-thione. Further, imino group-containing compounds can be used, too. Suitable examples thereof include the silver salts of benzotriazoles and derivatives thereof, such as the silver salts of alkyl-substituted benzotriazoles (e.g., methylbenzotriazole silver) and the silver salts of halogen-substituted benzotriazoles (e.g., 5-chlorobenzotriazole silver); the silver salts of 1,2,4-triazoles or 1-H-tetrazoles as described in U.S. Pat. No. 4,220,709; and the silver salts of imidazole and imidazole derivatives. Furthermore, various silver acetylides compounds as described, e.g., in U.S. Pat. Nos. 4,761,361 and 4,775,613 can be used, too.

The organic silver salts usable in the present invention have no particular restriction on their crystal forms. However, it is desirable for them to be needle-like crystals having a minor axis and a major axis. As for their grain size, on the other hand, the organic silver salts are required to have small grain sizes. This is because the inversely proportional relation between the grain size of silver salt and the covering power thereof, which is well known in the field of silver halide photosensitive materials, is valid for the present photothermographic material also. In other words, if the organic silver salt to function as the image-forming element in the present photothermographic material are large in grain size, high image density cannot be obtained because of their low covering power. Accordingly, it is desirable that the minor axis be from 0.01  $\mu\text{m}$  to 0.20  $\mu\text{m}$  and the major axis

be from 0.10  $\mu\text{m}$  to 5.0  $\mu\text{m}$ , and more desirable that the minor axis be from 0.01  $\mu\text{m}$  to 0.15  $\mu\text{m}$  and the major axis be from 0.10  $\mu\text{m}$  to 4.0  $\mu\text{m}$ . The size distribution among organic silver salt grains is preferably monodisperse. The term "monodisperse" as used herein means that, in the measurement of minor axis length and major axis length each, the standard deviation divided by the mean of measured values is, expressed in percentage, below 100%, preferably below 80%, particularly preferably below 50%. The measurements of organic silver salt grains can be examined by the observation of an organic silver salt dispersion under a transmission electron microscope. As for another method of examining the extent of monodispersion, there can be adopted the method of determining the standard deviation relating to the volume weighted-mean diameter of organic silver salt grains. Therein, it is desirable that the quotient of the standard deviation divided by the volume weighted-mean diameter (namely variation coefficient) be, expressed in percentage, below 100%, preferably below 80%, and more preferably below 50%. The standard deviation relating to the volume weighted-mean diameter can be determined, e.g., by irradiating an organic silver salt dispersed in a liquid with laser beam and determining the auto-correlation function of change in fluctuations of the scattered beam with the passage of time to obtain grain sizes (volume weighted mean diameter).

The amount of an organic silver salt used in the present invention, though it is optional, is preferably from 0.1 to 5 g/m<sup>2</sup>, and more preferably from 1 to 3 g/m<sup>2</sup>.

The reducing agent for organic silver salts may be any of materials capable of reducing silver ion to metallic silver, preferably organic ones. Although conventional photographic developing agents, such as phenidone, hydroquinone and catechol are useful, hindered phenols are preferred as the reducing agent. The reducing agent is required to be present in a proportion of 1 to 10 weight % in the image-forming layer. When the reducing agent is added to a layer except emulsion layers in a multilayer structure, it is a desirable tendency to add the reducing agent in a greater proportion, specifically a proportion of about 2 to 15 weight %.

For the organic silver salt-utilized photothermographic materials, a wide variety of reducing agents are disclosed. Specific examples thereof include amidoximes, such as phenylamidoxime, 2-thienylamidoxime and p-phenoxyphenylamidoxime; azines, such as 4-hydroxy-3, 5-dimethoxybenzaldehydeazine; the combinations of aliphatic carboxylic acid arylhydrazides with ascorbic acid, such as the combination of 2,2-bis(hydroxymethyl)propionyl- $\beta$ -phenylhydrazine with ascorbic acid; the combinations of polyhydroxybenzenes with hydroxylamines, reductones and/or hydrazines (e.g., the combination of hydroquinone with bis(ethoxyethyl)hydroxylamine, piperidino-hexose reductone or formyl-4-methylphenylhydrazine); hydroxamic acids, such as phenylhydroxamic acid, p-hydroxyphenylhydroxamic acid and  $\beta$ -anilinehydroxamic acid; the combinations of azines with sulfonamidophenols (e.g., the combination of phenothiazine with 2,6-dichloro-4-benzenesulfonamidophenol);  $\alpha$ -cyanophenylacetic acid derivatives, such as ethyl- $\alpha$ -cyano-2-methylphenylacetate, ethyl- $\alpha$ -cyanophenylacetate; bis- $\beta$ -naphthols, such as 2,2-

dihydroxy-1,1-binaphthyl, 6,6-dibromo-2,2-dihydroxy-1,1-binaphthyl and bis(2-hydroxy-1-naphthyl)methane; the combinations of bis- $\beta$ -naphthols with a 2,4-dihydroxybenzene derivative (such as 2,4-dihydroxybenzophenone or 2,4-dihydroxyacetophenone); 5-pyrazolones, such as 3-methyl-1-phenyl-5-pyrazolone; reductones, such as dimethylaminohexose reductone, anhydrodihydroaminohexose reductone and anhydrodihydropiperidonehexose reductone; sulfonamidophenol reducing agents, such as 2,6-dichloro-4-benzenesulfonamidophenol and p-benzenesulfonamidophenol; 2-phenylindane-1,3-dione and the like; chromans, such as 2,2-dimethyl-7-t-butyl-6-hydroxychroman; 1,4-dihydropyridines, such as 2,6-dimethoxy-3,5-dicarboethoxy-1,4-dihydropyridine; bisphenols, such as bis(2-hydroxy-3-t-butyl-5-methylphenyl)methane, 2,2-bis(4-hydroxy-3-methylphenyl)propane, 4,4-ethylidene-bis(2-t-butyl-6-methylphenol), 1,1-bis(2-hydroxy-3,5-dimethylphenyl)-3,5,5-trimethylhexane and 2,2-bis(3,5-dimethyl-4-hydroxyphenyl)propane; ascorbic acid derivatives, such as 1-ascorbyl palmitate and ascorbyl stearate; aldehydes and ketones of benzyl, biacetyl and the like; 3-pyrazolidones and certain indane-1,3-diones; and chromanols (e.g., tocopherols). Of these compounds, particularly preferable reducing agents are bisphenols and chromanols.

In addition to the foregoing ingredients, it is sometimes advantageous to the present photothermographic material to contain an additive known as "toning agent" for enhancing the image quality. For instance, the material for toning agent may be present in a proportion of 0.1 to 10 weight % to the total silver-holding components. The toning agent is a known ingredient in the photography, as described in U.S. Pat. Nos. 3,080,254, 3,847,612 and 4,123,282.

Specific examples of a toning agent include phthalimide and N-hydroxyphthalimide; cyclic imides, such as succinimide, pyrazoline-5-one, quinazolinone, 3-phenyl-2-pyrazoline-5-one, 1-phenylurazole, quinazoline and 2,4-thiazolidinedione; naphthalimides (e.g., N-hydroxy-1,8-naphthalimide); cobalt complexes (e.g., cobalthexamine trifluoroacetate); mercaptanes, such as 3-mercaptop-1,2,4-triazole, 2,4-dimercaptopyrimidine, 3-mercaptop-4,5-diphenyl-1,2,4-triazole and 2,5-dimercapto-1,3,4-thiadiazole; N-(aminomethyl)aryldicarboxyimides, such as (N,N-dimethylaminomethyl)phthalimide and N,N-(dimethylaminomethyl)-naphthalene-2,3-dicarboxyimide; blocked pyrazoles, isothiuronium derivatives and certain photodiscoloring agents (e.g., N,N-hexamethylenebis(1-carbamoyl-3,5-dimethylpyrazole), 1,8-(3,6-diazaoctane)bis(isothiuronium trifluoroacetate) and 2-(tribromomethylsulfonyl)benzothiazole; 3-ethyl-5[(3-ethyl-2-benzothiazolinidene)-1-methylethylidene]-2-thio-2,4-oxazolidinedione; phthalazinone, and phthalazinone derivatives or metal salts, e.g., 4-(1-naphthyl)phthalazinone, 6-chlorophthalazinone, 5,7-dimethoxyphthalazinone and 2,3-dihydro-1,4-phthalazinedione; the combinations of phthalazinone with phthalic acid derivatives (such as phthalic acid, 4-methylphthalic acid, 4-nitrophthalic acid and tetrachlorophthalic anhydride); phthalazine, and phthalazine derivatives or metal salts, e.g., 4-(1-naphthyl)phthalazine, 6-chlorophthalazine, 5,7-dimethoxyphthalazine and 2,3-dihydroxyphthalazine; the combinations of phthal-

zine with phthalic acid derivatives (such as phthalic acid, 4-methylphthalic acid, 4-nitrophthalic acid and tetrachlorophthalic anhydride); quinazolininedione, benzoxazine or naphthoxazine derivatives; rhodium complexes functioning as not only tone adjuster but also halide ion source for formation of silver halide in situ, such as ammonium hexachlororhodate(III), rhodium bromide, rhodium nitrate and potassium hexachlororhodate(III); inorganic peroxides and persulfates, e.g., ammonium peroxydisulfide and hydrogen peroxide; benzoxazine-2,4-diones, such as 1,3-benzoxazine-2,4-dione, 8-methyl-1,3-benzoxazine-2,4-dione and 6-nitro-1,3-benzoxazine-2,4-dione; pyrimidines (e.g., 2,4-dihydroxypyrimidine, 2-hydroxy-4-aminopyrimidine); asymmetric triazines; azauracil; and tetraazapentalene derivatives (e.g., 3,6-dimercapto-1,4-diphenyl-1H,4H-2,3a,5,6a-tetraazapentalene and 1,4-di(ochlorophenyl)-3,6-dimercapto-1H,4H-2,3a,5,6a-tetraazapentalene).

For the purpose of retarding or accelerating, that is, controlling the development, heightening the spectral sensitizing efficiency, enhancing the stability before and after the development and so on, a mercapto, disulfide or thione compound can be incorporated in the present photothermographic material.

The mercapto compound used in the present invention, though it may have any structure, is preferably a compound of represented by a formula Ar-SM or Ar-S-S-Ar, wherein M is a hydrogen atom or an alkali metal atom and Ar is an aromatic or condensed aromatic ring containing at least one nitrogen, sulfur, oxygen, selenium or tellurium atom. Such a heterocyclic aromatic ring is preferably a benzimidazole, naphthimidazole, naphthothiazole, benzoxazole, naphthoxazole, benzoselenazole, benzotellurazole, imidazole, oxazole, pyrazole, triazole, thiadiazole, tetrazole, triazine, pyrimidine, pyridazine, pyrazine, pyridine, purine, quinoline or quinazolinone ring. These rings each may have one or more of a substituent selected from among a halogen atom (e.g., Br and Cl), a hydroxy group, an amino group, a carboxyl group, an alkyl group (e.g., an alkyl group containing at least one, preferably 1 to 4, carbon atoms) and an alkoxy group (e.g., an alkoxy group containing at least one, preferably 1 to 4, carbon atoms). Specific examples of a mercapto-substituted heterocyclic aromatic compound include 2-mercaptopbenzimidazole, 2-mercaptopbenzoxazole, 2-mercaptopbenzothiazole, 2-mercaptop-5-methylbenzimidazole, 6-ethoxy-2-mercaptopbenzothiazole, 2,2'-dithiobis(benzothiazole), 3-mercaptop-1,2,4-triazole, 4,5-diphenyl-2-imidazolethiole, 2-mercaptopimidazole, 1-ethyl-2-mercaptopbenzimidazole, 2-mercaptopquinoline, 8-mercaptopurine, 2-mercaptop-4(3H)-quinazolinone, 7-trifluoromethyl-4-quinolinethiole, 2,3,5,6-tetrachloro-4-pyridinethiole, 4-amino-6-hydroxy-2-mercaptopyrimidine monohydrate, 2-amino-5-mercaptop-1,3,4-thiadiazole, 3-amino-5-mercaptop-1,2,4-triazole, 4-hydroxy-2-mercaptopyrimidine, 2-mercaptopyrimidine, 4,6-diamino-2-mercaptopyrimidine, 2-mercaptop-4-methylpyrimidine hydrochloride, 3-mercaptop-5-phenyl-1,2,4-triazole and 2-mercaptop-4-phenyloxazole, but these examples should not be construed as limiting the scope of the present invention.

It is desirable that the mercapto compound as recited above be incorporated in an emulsion layer in an amount of 0.001 to 1.0 mole, preferably 0.01 to 0.3 mole, per mole of silver.

## 25

The present photosensitive material can be provided with a surface protecting layer for the purpose of, e.g., preventing the adhesion of the image-forming layer. The surface protecting layer may be made from any adhesion preventing material. Suitable examples of an adhesion preventing material include wax, silica particles, a styrene-containing elastomeric copolymer (e.g., styrene-butadiene-styrene, or styrene-isobutylene-styrene), cellulose acetate, cellulose acetate butyrate, cellulose propionate, and mixtures of two or more thereof.

In the present emulsion layers and the protective layers therefor, the light-absorbing materials and the filter dyes as described in U.S. Pat. Nos. 3,253,921, 2,274,782, 2,527,583 and 2,956,879 can be used. The dyes incorporated can be mordanted as described, e.g., in U.S. Pat. No. 3,282,699. It is desirable for the filter dyes to be used in such an amount as to provide the absorbance of 0.1 to 3, preferably 0.2 to 1.5, at the wavelengths of exposure light.

The present emulsion layers and the protective layers therefor can contain a delustering agent, such as starch, titanium dioxide, zinc oxide, silica, and polymer beads including the beads described in U.S. Pat. Nos. 2,992,101 and 2,701,245. The matt degree on the emulsion side can be arbitrarily chosen so far as the star dust trouble does not occur, but it is desirably adjusted so that the Bekk smoothness ranges from 1,000 to 10,000 seconds, particularly from 2,000 to 10,000 seconds.

The binder for the present emulsion layers can be arbitrarily selected from well-known natural or synthetic resins, such as gelatin, polyvinyl acetal, polyvinyl chloride, polyvinyl acetate, cellulose acetate, polyolefin, polyester, polystyrene, polyacrylonitrile and polycarbonate. Of course, the binder may be selected from the copolymers and the terpolymers related to the above-recited ones. Specific examples of a polymer suitable for the binder include polyvinyl butyral, butyl ethyl cellulose, methacrylate copolymers, maleic anhydride copolymers, polystyrene and a butadiene-styrene copolymer. These polymers may be used as a mixture of two or more thereof, if needed. The polymers as recited above are used in an amount sufficient to hold ingredients therein. In other words, they are used in a range of amounts effective in functioning as binder. The effective amount range can be determined properly by persons skilled in the art. As for the measure in a case of holding at least an organic silver salt, it is desirable that the weight ratio of the binder to the organic silver halide be from 15:1 to 1:2, particularly from 8:1 to 1:1.

The present photothermographic material is preferably the so-called one-sided photosensitive material which has on one side of a support a photosensitive layer comprising at least one silver halide emulsion layer and on the other side a backing layer.

To the one-sided photosensitive material according to the present invention, a matting agent may be added for the purpose of making the travelling (conveying) properties better. In general, fine particles of water-insoluble organic or inorganic compounds are used as matting agent. Specifically, the matting agent used in the aforesaid photosensitive material may be any of the matting agents well known in the arts, including the organic matting agents described, e.g., in U.S. Pat. Nos. 1,939,213, 2,701,245,

## 26

2,322,037, 3,262,782, 3,539,344 and 3,767,448 and the inorganic matting agents described, e.g., in U.S. Pat. Nos. 1,260,772, 2,192,241, 3,257,206, 3,370,951, 3,523,022 and 3,769,020. More specifically, the organic compounds suitable for the matting agent include water-dispersable vinyl polymers, such as polymethylacrylate, polymethylmethacrylate, polyacrylonitrile, acrylonitrile- $\alpha$ -methylstyrene copolymer, polystyrene, styrene-divinylbenzene copolymer, polyvinyl acetate, polyethylene carbonate and polytetrafluoroethylene; cellulose derivatives, such as methyl cellulose, cellulose acetate and cellulose acetate propionate; starch derivatives, such as carboxystarch, carboxynitrophenyl starch and reaction products of urea, formaldehyde and starch; gelatins hardened with a known hardener; and gelatins hardened by coacervation to be formed into microencapsulated hollow particles. As for the inorganic compounds suitable for the matting agent, silicone dioxide, titanium dioxide, magnesium dioxide, aluminum oxide, barium sulfate, calcium carbonate, silver chloride and silver bromide desensitized by a known method, glass and diatomaceous earth are examples thereof. The matting agents recited above can be used as a mixture of two or more compounds of different kinds, if needed. The matting agent has no particular limitation on its size and shape, so that it may have any particle size. In practice, however, the particle size ranging from 0.1 to 30  $\mu$ m is advantageous to the matting agent used in the present invention. In addition, the particle size distribution of the matting agent used may be narrow or broad. On the other hand, the matting agent produces great influences on the haze and the surface gloss of a photosensitive material. Therefore, it is desirable that the particle size, the shape and the size distribution of the matting agent be adjusted so as to achieve the intended states of haze and surface gloss by properly choosing the production condition or mixing two or more of matting compounds.

As for the matt degree of a backing layer in the present invention, it is desirable that the backing layer have Bekk smoothness of from 10 to 250 seconds, preferably from 50 to 180 seconds.

In the present photosensitive material, it is desirable that the matting agent be incorporated in the outermost layers, layers functioning as the outermost layers, layers close to the outer surfaces, or layers acting as the so-called protective layers.

The binder suitable for the backing layer of the present photosensitive material is a transparent or translucent, colorless (in general) film-forming material, such as a natural polymer and a synthetic resin including homo- and copolymer. Specific examples thereof include gelatin, gum arabic, polyvinyl alcohol, hydroxyethyl cellulose, cellulose acetate, cellulose acetate butyrate, polyvinyl pyrrolidone, casein, starch, polyacrylic acid, polymethylmethacrylic acid, polyvinyl chloride, polymethacrylic acid, styrene-maleic anhydride copolymer, styrene-acrylonitrile copolymer, styrene-butadiene copolymer, polyvinyl acetals (e.g., polyvinyl formal, polyvinyl butyral), polyesters, polyurethanes, phenoxy resin, polyvinylidene chloride, polyepoxides, polycarbonates, polyvinyl acetate, cellulose esters and polyamides. The binder may be used in the form of solution in water or an organic solvent, or in the form of emulsion.

In the present invention, it is desirable that the backing layer have the absorption maximum of from 0.3 to 2 in the wavelength region of 750 to 1,400 nm, preferably IR absorption of 0.5 to 2, and have absorption of from 0.001 to smaller than 0.5 in the visible region. Further, it is preferable that the backing layer be an antihalation layer having the optical density of from 0.001 to lower than 0.3.

The dyes used as antihalation dyes in the present invention may be any compounds so far as they have the intended absorption in the region of 750 to 1,400 nm, are sufficiently low in visible absorption and provide the foregoing absorbance spectral form desired for the backing layer. As examples of such dyes, mention may be made of the compounds described in JP-A-07-13295 and U.S. Pat. No. 5,380,635, and the compounds described in JP-A-02-68539 (from page 13, left lower column, line 1, to page 14, left lower column, line 9) and JP-A-03-24539 (from page 14, left lower column, to page 16, right lower column). However, these examples should not be construed as limiting on the scope of the present invention.

The backside resistive heating layers as described in U.S. Pat. Nos. 4,460,681 and 4,374,921 can also be applied to the light-sensitve photothermographic image formation system.

The silver halide emulsions or/and the organic silver salts in the present invention can be further protected from the additional fog formation by the use of an antifogging agent, a stabilizer or a precursor of stabilizers to effect the stabilization for the lowering of sensitivity upon storage. Suitable examples of an antifogging agent, a stabilizer and a precursor of stabilizers which can be used alone or in combination include the thiazonium salts described in U.S. Pat. Nos. 2,131,038 and 2,694,716, the azaindenes described in U.S. Pat. Nos. 2,886,437 and 2,444,605, the mercury salts described in U.S. Pat. No. 2,728,663., the urazoles described in U.S. Pat. No. 3,287,135, the sulfocatechols described in U.S. Pat. No. 3,235,652, the oximes, the nitrones and the nitroindazoles described in British Patent 623,448, the polyvalent metal salts described in U.S. Pat. No. 2,839,405, the thiuronium salts described in U.S. Pat. No. 3,220,839, the palladium, platinum and gold salts described in U.S. Pat. Nos. 2,556,263 and 2,597,915, the halogen-substituted organic compounds described in U.S. Pat. Nos. 4,108,665 and 4,442,202, the triazines described in U.S. Pat. Nos. 4,128,557, 4,137,079, 4,138,365 and 4,459,350, and the phosphorus compounds described in U.S. Pat. No. 4,411, 985.

For the photosensitive layers in the present invention, polyhydric alcohols (e.g., glycerines and diols of the types described in U.S. Pat. No. 2,960,404), the fatty acids or their esters described in U.S. Pat. Nos. 2,588,765 and 3,121,060 and the silicone resins described in British Patent 955,061 can be used as plasticizer or lubricant.

In each of the constituent layers of the present material, including photosensitive, protective and backing layers, hardeners may be used. Specific examples of such hardeners include the polyisocyanates described in U.S. Pat. No. 4,281,060 and JP-A-06-208193, the epoxy compounds described in U.S. Pat. No. 4,791,042, and the vinylsulfone compounds described in JP-A-62-89048.

For the purpose of improving coating properties and antistatic properties, surfactants may be used in the present

invention. Any type of surfactant, including nonionic, anionic, cationic and fluorine-containing ones, can be used, if desired. As examples of a surfactant which can be properly used, mention may be made of the fluorine-containing high molecular surfactants described, e.g., in JP-A-62-170950 and U.S. Pat. No. 5,382,504, the fluorine-containing surfactants described, e.g., in JP-A-60-244945 and JP-A-63-188135, the polysiloxane surfactants described, e.g., in U.S. Pat. No. 3,885,965, and the polyalkylene oxides and the anionic surfactants described, e.g., in JP-A-06-301140.

In the present invention, hydrazine derivatives may be used. When the present invention uses a hydrazine derivative, the hydrazine derivative can be a compound represented by the formula (I) illustrated in Japanese Patent Application No. 6-47961 (corresponding to JP-A-7-287335). Specifically, the compounds exemplified as I-1 to I-53 in the reference cited above can be used.

Besides the above compounds, the following hydrazine derivatives can also be used to advantage: They include the compounds of formula (Ka-1) illustrated in JP-B-06-77138, specifically the compounds illustrated at pages 3-4 of the said gazette; the compounds of formula (I) illustrated in JP-B-06-93082, specifically Compounds 1 to 38 illustrated at pages 8-18 of the said gazette; the compounds of formula (4), (5) or (6) illustrated in JP-A-06-230497, specifically Compounds 4-1 to 4-10, Compounds 5-1 to 5-42 and Compounds 6-1 to 6-7 illustrated at pages 25-26, pages 28-36 and pages 39-40, respectively, of the said gazette; the compounds of formula (1) or (2) illustrated in JP-A-06-289520, specifically Compounds 1-1) to 1-17) and Compound 2-1) illustrated at pages 5-7 of the said gazette; the compounds of formula (Ka-2) or (Ka-3) illustrated in JP-A-06-313936, specifically the compounds illustrated at pages 6-19 of the said gazette; the compounds of formula (Ka-1) illustrated in JP-A-06-313951, specifically the compounds illustrated at pages 3-5 of the said gazette; the compounds of formula (I) illustrated in JP-A-07-5610, specifically Compounds I-1) to I-38) illustrated at pages 5-10 of the said gazette; the compounds of formula (II) illustrated in JP-A-07-77783, specifically Compounds II-1) to II-102) illustrated at pages 10-27 of the said gazette; the compounds of formula (H) or (Ha) illustrated in JP-A-07-104426, specifically Compounds H-1 to H-44 illustrated at pages 8-15 of the said gazette; the compounds described in JP-A-9-22082 which are characterized by containing anionic groups in the vicinity of their respective hydrazino groups or nonionic groups forming intramolecular hydrogen bonding together with hydrogen atoms of their respective hydrazino groups, especially the compounds of formula (A), (B), (C), (D), (E) or (F) with specific examples including Compounds N-1 to N-30; and the compounds of formula (1) illustrated in JP-A-9-22082, specifically Compound D-1 to D-55 illustrated in the said gazette.

In using a nucleating agent of hydrazine type in the present invention, the nucleating agent may be dissolved in an appropriate water-miscible organic solvent, such as an alcohol (e.g., methanol, ethanol, propanol, a fluorinated alcohol), a ketone (e.g., acetone, methyl ethyl ketone), dimethylformamide, dimethyl sulfoxide or methyl cellosolve.

On the other hand, an emulsified dispersion of nucleating agent may be prepared using a well-known method, which

comprises a step of dissolving the agent in an oil, such as dibutyl phthalate, tricresyl phosphate, glyceryl triacetate or diethyl phthalate, admixed with an auxiliary solvent such as ethyl acetate or cyclohexanone, if needed, and a step of mechanically emulsifying and dispersing the dissolved agent. Also, the powder of a hydrazine derivative may be dispersed into water with a ball mill, a colloid mill or ultrasonic waves according to the method known as solid dispersion method.

The nucleating agent of hydrazine type may be added to any of silver halide emulsion layers and other hydrophilic colloid layers arranged on the emulsion side of the support. In the present invention, however, it is desirable for the nucleating agent to be added to a silver halide emulsion layer or the hydrophilic colloidal layer adjacent thereto.

It is desirable in the present invention that the amount of the nucleating agent added be from 1  $\mu$ mole to 10 mmole, preferably from 10  $\mu$ mole to 5 mmole, particularly preferably from 20  $\mu$ mole to 5 mmole, per mole of silver halide.

The addition of a mercury(II) salt as antifogging agent to an emulsion layer, though not essential to the present invention, is sometimes favorable for the present invention. The mercury(II) salts suitable for the above purpose are mercury acetate and mercury bromide. The proportion of the light-sensitive silver halide used in the present invention is generally from 0.75 to 25 mole %, preferably from 2 to 20 mole %, to the organic silver salt.

The photothermographic emulsions according to the present invention can be coated on a wide variety of supports. Typical examples of a usable support include a polyester film, a polyester film provided with a subbing layer, a polyethylene terephthalate film, a polyethylene naphthalate film, a cellulose nitrate film, a cellulose ester film, a polyvinyl acetal film, a polycarbonate film and resinous materials related thereto, and glass, paper and metal as well. Of these materials, flexible support materials, especially paper supports partially acetylated or coated with baryta and/or an  $\alpha$ -olefin polymer, preferably the polymer of an  $\alpha$ -olefin containing 2 to 10 carbon atoms, such as polyethylene, polypropylene or an ethylene-butene copolymer, are representative support materials. The support used in the present invention, though may be any of transparent and opaque ones, is preferably transparent.

The photosensitive material according to the present invention may have an antistatic or conductive layer, such as a layer containing a soluble salt (e.g., a chloride, a nitrate), an evaporated metal layer, or a layer containing the ionic polymer as described in U.S. Pat. Nos. 2,861,056 and 3,206,312 or the insoluble inorganic salt as described in U.S. Pat. No. 3,428,451.

In forming color images with a photothermographic material according to the present invention, the method described in JP-A-07-13295 (from page 10, left column, line 43, to page 11, left column, line 40) can be adopted. The stabilizers for color dye images formed therein are described in British Patent 1,326,889 and U.S. Pat. Nos. 3,432,300, 3,698,909, 3,574,627, 3,573,050, 3,764,337 and 4,042,394.

The photothermographic emulsions according to the present invention can be coated by any of various coating operations, including a dip coating operation, an air knife coating operation, a flow coating operation and an extrusion

coating operation using the hopper described in U.S. Pat. No. 2,682,294. Two or more of those emulsions can be coated simultaneously using the method described in U.S. Pat. No. 2,761,791 or British Patent 837,095, if desired.

In the photothermographic material according to the present invention can be comprised additional layers, such as a dye-receiving layer for receiving transferred dye images, an opacified layer required in the case of reflection printing, a protective top coat layer and a primer layer known in the heat- and light-sensitive photography. In this case, it is desirable that the functional layers necessary for image formation, including an image-receiving layer, be integrated into the present photosensitive material to enable the photosensitive material to form images by itself.

The photosensitive materials according to the present invention, though they may be developed in any manner, are generally developed by raising the temperature thereof after imagewise exposure. The suitable temperature for development is from 80 to 250° C., preferably from 100 to 140° C. As for the development time, the range of 1 to 180 seconds is appropriate and that of 10 to 90 seconds is more appropriate.

The photosensitive materials according to the present invention can be exposed by any method. As the light source for exposure, however, it is desirable to use laser beams. The laser beams suitable for the present invention are beams generated by gas laser, YAG laser, dye laser, semiconductor laser or the like. Also, the combination of semiconductor laser with a second harmonic wave generating device can be used.

The present invention will now be illustrated in more detail by reference to the following examples, but these examples should not be construed as limiting on the scope of the invention in any way.

#### EXAMPLE 1

##### Preparation of Silver Halide Grains

A solution containing 22 g of phthaloylated gelatin and 30 mg of potassium bromide in 700 ml of water was adjusted to pH 5.0 at 35° C., and thereto 159 ml of a water solution containing 18.6 g of silver nitrate and a water solution containing potassium bromide and potassium iodide in a ratio of 92:8 by mole were added over a 10-minute period as the pAg was kept at 7.7 in accordance with the controlled double jet method. Thereto, 476 ml of a water solution containing 55.4 g of silver nitrate and a water solution containing 9  $\mu$ mole/l of dipotassium hexachloroiridate and 1 mole/l of potassium bromide were further added over a 30-minute period as the pAg was kept at 7.7 in accordance with the controlled double jet method. Then, the pH of the resultant solution was lowered to cause flocculation, thereby effecting a desalting treatment. The thus desalting matter was admixed with 0.10 g of phenoxyethanol, and adjusted to pH 5.9 and pAg 8.2 to prepare silver iodobromide grains (cubic grains having the iodide content of 2 mole % on the average and 8 mole % in the core part, the average size of 0.05  $\mu$ m, the projected area variation coefficient of 8%, and the (100) face proportion of 87%).

The silver halide grains thus obtained were heated up to 60° C., and thereto were added 85  $\mu$ mole/mole silver of

**31**

sodium thiosulfate, 11  $\mu$ mole/mole silver of 2,3,4,5,6-pentafluorophenylidiphenylphosphine selenide, 15  $\mu$ mole/mole silver of Tellurium Compound 1 illustrated below, 2  $\mu$ mole/mole silver of chloroauric acid and 200  $\mu$ mole/mole silver of thiocyanic acid. The resultant mixture was ripened for 150 minutes, and then quenched rapidly to 30° C., thereby preparing a silver halide emulsion.

## Preparation of Organic Acid-Silver Salt Emulsion

Stearic acid, arachidic acid and behenic acid in amounts of 1.3 g, 0.5 g and 8.5 g, respectively, and 300 ml of distilled water were mixed for 15 minutes at 90° C., and thereto 31.1 ml of an aqueous 1N-NaOH solution was added over a 15-minute period with vigorous stirring. Then, the admixture was cooled to 30° C., and thereto 7 ml of an aqueous 1N-H<sub>3</sub>PO<sub>4</sub> solution was added. Further thereto, 9 mg of N-bromosuccinimide was added with more vigorous stirring. The resultant mixture was admixed with the previously prepared silver halide grains in the amount of 2.5 mmole. Thereto, 25 ml of an aqueous 1N-AgNO<sub>3</sub> solution was added over a 2-minute period, and the stirring was continued for 90 minutes. Thereafter, the solid matter was filtered with suction, and washed. This operation was repeated till the conductivity of the filtrate became 30  $\mu$ S•cm. The thus obtained solid matter was admixed with 37 g of a 1.2 weight % butyl acetate solution of polyvinyl acetate, and stirred. After finish the stirring, the admixture was allowed to stand, and thereby it was separated into an oil layer and a water layer. The water layer was removed together with the salts contained therein to isolate the oil layer. To the thus obtained oil layer, 20 g of a 2.5 weight % 2-butanone solution of polyvinyl butyral (Denka Butyral #3000-K, commercial name, a product of Electro Chemical Industry Co., Ltd.) was added with stirring. Further thereto, 0.1 mmole of bromopyridinium perbromide and 0.1 mmole potassium bromide

**32**

dihydrate were added together with 0.7 g methanol. Furthermore thereto, 40 g of 2-butanone and 7.8 g of polyvinyl butyral (PBV B-76, commercial name, a product of Monsanto Co.) were added, and subjected to a dispersing operation with a homogenizer. Thus, an organic acid-silver salt emulsion (needle grains having the average breadth of 0.04  $\mu$ m, the average length of 1  $\mu$ m and the variation coefficient of 27%) was obtained.

## 10 Preparation of Coating Composition for Emulsion Layer

To the organic acid-silver salt emulsion obtained above, the ingredients described below were added in the following amounts, respectively, per mole of silver to prepare Coating Composition A for an emulsion layer. Specifically, 10 mg of sodium phenylthiosulfonate, 70 mg of the present Cyanine Dye 1, 2 g of 2-mercaptop-5-methylbenzimidazole, 21.5 g of 4-chlorobenzophenone-2-carboxylic acid, 580 g of 2-butanone and 220 g of dimethylformamide were admixed at 25° C. with stirring. The resulting admixture was allowed to stand for 3 hours. Thereto, 8 g of 5-tribromomethylsulfonyl-2-methylthiadiazole, 6 g of 2-tribromomethylsulfonylbenzothiazole, 5 g of 4,6-ditrichloromethyl-2-phenyltriazine, 2 g of Disulfide Compound 1 illustrated below, 155 g of 1,1-bis(2-hydroxy-3,5-dimethylphenyl)-3,5,5-trimethylhexane, 5 g of tetrachlorophthalic acid, 1.1 g of a fluorine-containing surfactant (Megafac F-176P, commercial name, a product of Dai-Nippon Ink & Chemicals, Inc.), 590 g of 2-butanone and 10 g of methyl isobutyl ketone were added with stirring.

20 Other Coating Compositions B to E were prepared in the same manner as described above, except that the present Cyanine Dyes 2 to 3 and Comparative Dyes 1 to 2 in their 25 respective amounts equimolar with the present Cyanine Dye 1 were used respectively in place of the present Cyanine Dye 1.

Tellurium Compound 1



Disulfide Compound 1



Comparative Dye 1



-continued

Comparative Dye 2



Preparation of Coating Composition for Protective Layer on Emulsion Side

In a mixture of 3,070 g of 2-butanone with 30 g of ethyl acetate were dissolved 75 g of cellulose acetate butyrate (CAB171-15S, commercial name, a product of Eastman Chemical Co., Ltd.), 5.7 g of 4-methylphthalic acid, 1.5 g of tetrachlorophthalic anhydride, 12 g of phthalazine, 0.3 g of Megafac F-176P, 2 g of very spherical silica having the average size of 3  $\mu\text{m}$  (Silidex H31, commercial name, a product of Dokai Chemical Co., Ltd.) and 6 g of polyisocyanate (Sumidur N3500, commercial name, a product of Sumitomo Bayer Urethane Co., Ltd.), thereby preparing a coating composition.

Composition to be coated on Back Side

A calcium compound (Calcium Compound 1) was produced in the following manner: To 1 l of an ethanol solution containing 0.08 mole of 3,5-di-tert-butylcatechol were added 167 ml of a water solution containing 0.019 mole of calcium chloride and 125 ml of 25% aqueous ammonia. Thereinto, air was bubbled for 3 hours at room temperature to precipitate the crystals of bis[2-(3,5-di-tert-butyl-*o*-benzoquinone monoimide)-4,6-di-tert-butylphenolato] calcium(II) (Calcium Compound 1).

To a mixture of 500 g of 2-butanone with 500 g of 2-propanol, 12 g of polyvinyl butyral (Denka Butyral #4000-2, commercial name, a product of Electro Chemical Industry Co., Ltd.), 12 g of cellulose acetate butyrate

(CAB381-20, commercial name, a product of Eastman Chemical Co., Ltd.), 120 mg of Dye 1, 300 mg of Calcium Compound 1, 350 mg of Dye 2, 5 mg of Dye 3, 0.4 g of very spherical silica having the average size of 12  $\mu\text{m}$  (Silidex H121, commercial name, a product of Dokai Chemical Co., Ltd.), 0.4 g of very spherical silica having the average size of 5  $\mu\text{m}$  (Silidex H51, commercial name, a product of Dokai Chemical Co., Ltd.), 0.1 g of Magafax F-176P and 2 g of Sumidur N3500 were added with stirring to mix them homogeneously. Thus, a back-side coating composition was prepared.

Preparation of Photosensitive Material

The Coating Compositions A to E prepared above for emulsion layers were each coated on a 175  $\mu\text{m}$ -thick, blue dye-tinged polyethylene terephthalate support at a silver coverage of 2.3 g/m<sup>2</sup>, and then the back-side coating composition prepared above was coated on the side opposite the emulsion layer so that the coating had an optical density of 0.7 at 810 nm. Further, the foregoing coating composition for protective layer was coated on the emulsion layer so that the protective layer formed had a dry thickness of 2  $\mu\text{m}$ . The thus obtained photosensitive materials A to E each had a smoothness of 1,000 seconds on the emulsion side and a smoothness of 80 seconds on the back side (wherein the smoothness values were determined as Bekk smoothness by the Ohken-type smoothness measurement described in J. TAPPI paper and pulp testing method No. 5).

Dye 1

 $\text{BF}_4^-$



Dye 2



Dye 3



#### Evaluation of Photographic Properties

The photosensitive materials A to E were each exposed by means of a laser sensitometer equipped with a 810 nm diode, and processed (developed) at 120° C. for 15 seconds. The thus obtained images were each evaluated by the measurement with a densitometer. Therein, the values of D<sub>min</sub> and sensitivity (the reciprocal of ratio of an exposure amount providing the density higher than D<sub>min</sub> by 1.0) were determined. Additionally, the sensitivities shown in Table 1 are relative values, with the photosensitive material A being taken as 100.

#### Evaluation of Aging Characteristics upon Storage

Each of the photosensitive materials A to E was allowed to stand for one day under the condition of 25° C.-50% RH.

Ten sheets of each photosensitive material were sealed in a bag made of a moisture-proofing material and further packed in a veneered case having the volume of 35.1 cm×26.9 cm<sup>55</sup> x 3.0 cm, and stored for 5 days at 50° C. Thus, forcibly aged samples were prepared. In addition, a reference standard of each sample was prepared as follows: Other ten sheets of each photosensitive material were subjected to the same treatment as described above, except that the storage temperature was changed to 4° C. The thus prepared forcibly aged samples and reference samples were each subjected to the same processing operations as in the evaluation of the photographic properties, and examined for fog density. The natural aging characteristics were evaluated by an increase rate in fog.

The increase rate in fog is defined by the following equation:

$$\text{Increase rate in fog} = \frac{[(\text{fog density of forcibly aged sample}) - (\text{fog density of reference sample})] \times (\text{maximum density of reference sample}) - (\text{support density})]}{100}$$

Accordingly, the lower the increase rate in fog, the better the natural aging characteristics.

#### Evaluation of Image Storage Characteristics under Exposure to Light

Each photosensitive material which had been exposed and developed under the same conditions as in the evaluation of photographic properties was fixed on the inside of a glass window exposed direct to the sun, and allowed to stand for 1 month. Then, the image appearance was evaluated by visual observation according to the following criterion:

Ⓐ . . . practically no change.

Ⓑ . . . slight change in tone but negligible.

Ⓒ . . . color change in the image area but practically allowable.

Ⓓ . . . color change and density increase in the D<sub>min</sub> area, and so improper.

#### Evaluation of Image Storage Characteristics under Exposure to Heat in the Dark

Each photosensitive material which had been exposed and developed under the same conditions as in the evaluation of photographic properties was allowed to stand for 1 month at 40° C. under a light-shielded condition. Then, the image appearance was evaluated by visual observation according to the following criterion:

Ⓐ . . . practically no change.

Ⓑ . . . slight change in tone but negligible.

Ⓒ . . . color change in the image area but practically allowable.

Ⓓ . . . color change and density increase in the D<sub>min</sub> area, and so improper.

The results of the aforementioned characteristics evaluations are shown in Table 1. As can be seen from Table 1, high sensitivity, low D<sub>min</sub>, excellent aging characteristics and excellent image storage characteristics were achieved only within the scope of the present invention.

TABLE 1

| Photo-sensitive |             | Aging            |                              | Image Storage Characteristics |                                    |            |
|-----------------|-------------|------------------|------------------------------|-------------------------------|------------------------------------|------------|
| material Name   | Sensitivity | D <sub>min</sub> | characteristics upon storage | under exposure to light       | under exposure to heat in the dark | Note       |
| A               | 100         | 0.1              | 1                            | Ⓐ                             | Ⓐ                                  | invention  |
| B               | 115         | 0.20             | 2                            | Ⓐ                             | Ⓐ                                  | invention  |
| C               | 110         | 0.20             | 1                            | Ⓐ                             | Ⓐ                                  | invention  |
| D               | 20          | 0.20             | 20                           | 0                             | △                                  | comparison |
| E               | 80          | 0.25             | 90                           | x                             | x                                  | comparison |

## EXAMPLE 2

## Preparation of Organic Acid-Silver Salt Emulsion

Behenic acid in the amount of 840 g and stearic acid in the amount of 95 g were added to 12 liter of water, and kept at 90° C. Thereto, a solution containing 48 g of sodium hydroxide and 63 g of sodium carbonate in 1.5 liter of water was added, and stirred for 30 minutes. After cooling to 50°

C., the resultant solution was admixed with 1.1 liter of a 1% water solution of N-bromosuccinimide. Thereto, 2.3 liter of a 17% water solution of silver nitrate was added little by little with stirring. Further, the solution temperature was lowered to 35° C., and 1.5 liter of a 2% water solution of potassium bromide was added over a 2-minute period with stirring. The resultant mixture was stirred for 30 minutes, and then admixed with 2.4 liter of a 1% water solution of N-bromosuccinimide. To this aqueous mixture, 3,300 g of a 1.2 weight % butyl acetate solution of polyvinyl acetate was added with stirring, and allowed to stand for 10 minutes to result in separation into two layers. The water layer thus separated was removed, and the gel remaining was washed twice with water. The thus obtained mixture of silver behenate/stearate gel with silver bromide was dispersed into 1,800 g of a 2.6% isopropanol solution of polyvinyl butyral (Denka Butyral #3000-K, commercial name, a product of Electro Chemical Industry Co., Ltd.), and further dispersed with a mixture of 600 g of polyvinyl butyral (Denka Butyral #4000-2, commercial name, a product of Electro Chemical Industry Co., Ltd.) and 300 g of isopropanol. Thus, an organic acid-silver salt emulsion (needle grains having the average breadth of 0.05 μm, the average length of 1.2 μm and the variation coefficient of 26%) was obtained.

## Preparation of Coating Composition for Emulsion Layer

To the organic acid-silver salt emulsion obtained above, the ingredients described below were added in the following amounts, respectively, per mole of silver to prepare Coating Composition W for an emulsion layer. Specifically, 10 mg of sodium phenylthiosulfonate, 70 mg of the present Cyanine Dye 2, 2 g of 2-mercapto-5-methylbenzimidazole, 21.5 g of 4-chlorobenzophenone-2-carboxylic acid, 580 g of 2-butanone and 220 g of dimethylformamide were admixed at 25° C. with stirring. The resulting admixture was allowed to stand for 3 hours. Thereto, 8 g of 5-tribromomethylsulfonyl-2-methylthiadiazole, 6 g of 2-tribromomethylsulfonylbenzothiazole, 5.1 g of 4,6-ditrichloromethyl-2-phenyltriazine, 2 g of Disulfide Compound 1, 160 g of 1,1-bis(2-hydroxy-3,5-dimethylphenyl)-3,5,5-trimethylhexane, 5 g of tetrachlorophthalic acid, 2.3 g of Hydrazine Derivative a, 1.1 g of a fluorine-containing

surfactant (Megafac F-176P, commercial name, a product of Dai-Nippon Ink & Chemicals, Inc.), 590 g of 2-butanone and 10 g of methyl isobutyl ketone were added with stirring.

Other Coating Compositions X, Y, Z and R were prepared in the same manner as described above, except that the present Cyanine Dyes 8, 14 and 30 and Comparative Dye 1 in their respective amounts equimolar with the present

Cyanine Dye 2 were used respectively in place of the present Cyanine Dye 2.

Preparation of Coating Composition for Protective Layer on Emulsion Side

In a mixture of 3,070 g of 2-butanone with 30 g of ethyl acetate were dissolved 75 g of cellulose acetate butyrate (CAB171-15S, commercial name, a product of Eastman Chemical Co., Ltd.), 5.7 g of 4-methylphthalic acid, 1.5 g of tetrachlorophthalic anhydride, 13 g of phthalazine, 0.3 g of Megafac F-176P, 2 g of very spherical silica having the average size of 3  $\mu\text{m}$  (Silidex H31, commercial name, a product of Dokai Chemical Co., Ltd.) and 7 g of polyisocyanate (Sumidur N3500, commercial name, a product of Sumitomo Bayer Urethane Co., Ltd.), thereby preparing a coating composition.

Preparation of Support having Backing Layer

A 100  $\mu\text{m}$ -thick polyethylene terephthalate film provided on both sides with a moisture-proofing undercoat comprising polyvinylidene chloride (a support) was covered with the same backing layer as in Example 1.

On the side opposite to the backing layer, the support was coated with each of the Coating Compositions W, X, Y, Z and R prepared above for emulsion layer so as to have a silver coverage of 2  $\text{g}/\text{m}^2$ , and further with the foregoing coating composition for protective layer on the emulsion side so that the protective layer formed had a dry thickness of 2  $\mu\text{m}$ . Thus, photosensitive materials W, X, Y, Z and R were obtained.



Hydrazine Derivative a

Evaluation of Photographic Properties of Hard Photosensitive Material

The photosensitive materials W, X, Y, Z and R were each exposed by means of a laser sensitometer equipped with a 820 nm diode, and processed (developed) at 115°C. for 25 seconds. The thus obtained images were each evaluated by the measurement with a densitometer. Therein, the values of Dmin and sensitivity (the reciprocal of ratio of an exposure amount providing the density higher than Dmin by 3.0) were determined. Additionally, the sensitivities shown in Table 2 are relative values, with the photosensitive material W being taken as 100. Further, each photosensitive material was examined for gradient  $\gamma$ , which was defined as the slope of a straight line connecting the points on the characteristic curve corresponding to the densities 0.3 and 3.0, respectively.

TABLE 2

| Photosensitive Material Name | Sensitivity | Dmin | $\gamma$ | note      |
|------------------------------|-------------|------|----------|-----------|
| W                            | 100         | 0.19 | 15       | invention |
| X                            | 112         | 0.20 | 12       | invention |
| Y                            | 107         | 0.18 | 15       | invention |

TABLE 2-continued

| Photosensitive Material Name | Sensitivity | Dmin | $\gamma$ | note       |
|------------------------------|-------------|------|----------|------------|
| Z                            | 110         | 0.20 | 13       | invention  |
| R                            | 30          | 0.25 | 4        | comparison |

As can be seen from Table 2, high sensitivity, low Dmin and high contrast were attained only within the scope of the present invention.

The photothermographic materials according to the present invention have low fog density, high sensitivity, high contrast and excellent storage characteristics before and after processing operations.

What is claimed is:

1. A photothermographic material comprising on at least one side of a support, a binder, an organic silver salt, a reducing agent for silver ions and light-sensitive silver halide grains, said photothermographic material comprising a cyanine dye represented by the following formula (I):



(X)i

wherein  $Z_1$  and  $Z_2$  each represents an atomic group for completing a benzene or naphthalene ring;  $Y_1$  and  $Y_2$  each represents O, S, Se or NR, wherein R is an alkyl group;  $R_1$  and  $R_2$  each represents an alkyl group;  $R_3$ ,  $R_4$ ,  $R_5$ ,  $R_6$ ,  $R_7$ ,  $R_8$  and  $R_9$  each represent a hydrogen atom or a substituent group,  $R_4$  and  $R_6$ ,  $R_5$  and  $R_7$ , or  $R_6$  and  $R_8$  may be combined with each other to form a 5- or 6-membered ring, and  $R_4$ ,  $R_6$  and  $R_8$  may be combined with each other to form a condensed ring in which two 6-membered rings are fused; X represents a counter ion for adjusting the charge balance; i represents 0 or 1; provided that  $R_1$ ,  $R_2$ ,  $R_3$ ,  $R_4$ ,  $R_5$ ,  $R_6$ ,  $R_7$ ,  $R_8$ ,  $R_9$ , R,  $Z_1$  or  $Z_2$  has as a substituent at least one thiienyl group.

2. A photothermographic material according to claim 1, said light-sensitive silver halide grains being spectrally sensitized in the wavelength region of 750 to 1,400 nm.

3. A photothermographic material according to claim 1, wherein said at least one thiienyl group exists as a substituent for a group represented by  $Z_1$ ,  $Z_2$ ,  $R_1$  or  $R_2$ .

4. A photothermographic material according to claim 1, wherein  $Z_1$  and  $Z_2$  each represents an atomic group for completing a benzene ring having a thiienyl group.

5. A photothermographic material according to claim 1, wherein at least one of  $Y_1$  and  $Y_2$  is S and the remainder is O or S.

6. A photothermographic material according to claim 1, wherein  $Y_1$  and  $Y_2$  each represents S.

7. A photothermographic material according to claim 1, wherein  $R_1$  and  $R_2$  each represents an unsubstituted alkyl group having 2 to 6 carbon atoms or a carboxyalkyl group.

8. A photothermographic material according to claim 1, wherein  $R_4$  and  $R_6$ , or  $R_6$  and  $R_8$  are combined with each other to form a 5- or 6-membered ring.

41

9. A photothermographic material according to claim 1, wherein  $Z_1$  and  $Z_2$  each represents an atomic group for completing a benzene ring having a thienyl group; at least one of  $Y_1$  and  $Y_2$  is S and the remainder is O or S;  $R_1$  and  $R_2$  each represents an unsubstituted alkyl group having 2 to 6 carbon atoms or a carboxyalkyl group; and  $R_4$  and  $R_6$ , or  $R_6$  and  $R_8$  are combined with each other to form a 5- or 6-membered ring.

**10.** A photothermographic material according to claim 1, wherein said cyanine dye is used in an amount of from  $10^{-6}$  to 1 mole per mole of silver halide. 10

42

11. The photothermographic material of claim 1, wherein R<sub>1</sub> and R<sub>2</sub> are each independently selected from the group consisting of a straight chain unsubstituted alkyl group, carboxyalkyl group, alkylthioalkyl group, thienylalkyl group, and an arylthioalkyl group.

12. The photothermographic material of claim 1, wherein  $R_3$ – $R_9$  are hydrogen atoms.

13. The photothermographic material of claim 1, wherein said cyanine dye is selected from the group consisting of:



-continued

I<sup>-</sup>CH<sub>3</sub>-C<sub>6</sub>H<sub>5</sub>-SO<sub>3</sub><sup>-</sup>I<sup>-</sup>I<sup>-</sup>I<sup>-</sup>

-continued

I<sup>-</sup>I<sup>-</sup>I<sup>-</sup>I<sup>-</sup>

-continued



and



14. The photothermographic material of claim 1, wherein said organic silver salt is used in an amount from 0.1 to 3 g/m<sup>2</sup>.